

1

3,345,173  
**STABILIZED PHOTOGRAPHIC PREHARDENER  
COMPOSITIONS**

Howard E. Munro, Rochester, N.Y., assignor to Eastman  
Kodak Company, Rochester, N.Y., a corporation of  
New Jersey  
No Drawing. Filed July 14, 1965, Ser. No. 472,048  
3 Claims. (Cl. 96—50)

This invention relates to photographic prehardener compositions which have been stabilized to prevent formation of peroxide compounds during storage.

It is known that photographic films and papers can be processed to provide useful photographic records in shorter periods of time than normal by carrying out the conventional processing steps at elevated temperatures, such as 80 to 150° F. However, such high temperature processing requires prehardening of the material to be processed so that undue softening of the colloid binder layers does not occur and scuffing and marking of the colloid binder layers is minimized.

One very useful means of accomplishing such prehardening is described in the copending application of Baden, Bard and Seemann U.S. Ser. No. 321,323, filed Nov. 4, 1963, now Patent No. 3,294,536. The prehardener compositions described in the Baden et al. application contain a dialkoxytetrahydrofuran, such as dimethoxytetrahydrofuran, diethoxytetrahydrofuran, etc., as the active hardening ingredient. Such materials contain the alkoxy groups as substituents on the carbon atoms adjacent to the oxygen atoms. When added to solutions having a low pH, e.g., 2-5, these furan compounds decompose to provide succinaldehyde, which is a useful hardening agent, particularly for gelatin layers of the type conventionally used in photography, either as a colloid binder for the light-sensitive silver halide, or in a protective overcoat layer. The succinaldehyde precursor can be used alone to perform hardening or can be used in conjunction with other hardening compounds, particularly formaldehyde.

While the dialkoxytetrahydrofuran compounds are quite useful for prehardening purposes, they suffer from the disadvantage of forming peroxides upon storage. For example, 2,5-dimethoxytetrahydrofuran is quite useful in prehardening color films and papers, particularly those containing color-forming compounds or couplers within the light-sensitive layers, but this compound produces undesirable peroxide compounds if stored for any appreciable time before use, and it is obvious that these peroxide compounds, if allowed to increase sufficiently in amount, will cause disastrous results when the photographic material is prehardened in a bath containing a contaminated tetrahydrofuran compound.

I have found that the deleterious formation of peroxide compounds in dialkoxytetrahydrofuran compositions can be completely eliminated or substantially reduced if small amounts of a butylated phenol compound containing an alkoxy radical or an alkyl radical in the position para to the hydroxyl group is added to the tetrahydrofuran compounds before storage. For example, amounts as small as 0.025% by weight, based on the tetrahydrofuran compound, have been found to have remarkable results in preventing such undesired peroxide formation. The quantity of phenol compound added as a stabilizing agent can vary considerably, depending upon the purity of the tetrahydrofuran compound, the ultimate use for the composition, etc. In general, only small amounts are required, but I have found that from about 0.025-0.40% by weight, based on the weight of the tetrahydrofuran compound is sufficient to stabilize such tetrahydrofuran compounds for substantial periods of time. Larger amounts of phenol stabilizers can be used, although ordinarily there is no advantage in doing so.

2

It is, therefore, an object of my invention to provide stabilized photographic prehardener compositions containing a dialkoxytetrahydrofuran compound. Another object is to provide butylated phenol compounds containing a substituent para to the hydroxyl group, which are particularly useful as stabilizing materials. Another object is to provide aqueous prehardening compositions which are particularly useful in treating photographic color films and papers so that they can be processed at elevated temperatures without adverse effects. Other objects will become apparent from the following description and examples.

Particularly useful butylated phenol compounds for the purposes of my invention comprise 2,6-di-tertiary butyl-p-cresol, butylated hydroxyanisole (BHA), etc. These particular phenol compounds are particularly useful since they are markedly effective in controlling peroxide formation, while at the same time they have little or no deleterious photographic effects, which might become apparent in using dialkoxytetrahydrofuran compounds in photographic prehardening solutions.

The stabilizing compounds of my invention can be intimately mixed with the dialkoxytetrahydrofuran compounds in any suitable manner, since such small amounts are employed. For example, a small amount of the stabilizer dissolved in a suitable solvent, such as propylene glycol, can be added to the dialkoxytetrahydrofuran compound and the mixture run through any suitable mixing apparatus, such as a ball mill or the like. In the above described manner, 2,5-dimethoxytetrahydrofuran was stabilized by the addition thereto of 0.01% of 2,6-di-tertiarybutyl-p-cresol. No peroxide formation was evident at the end of one year. This material containing both the tetrahydrofuran compound (DMTF) and the cresol compound was used in the following examples:

*Example 1*

800 ml. of water at 90° F. was used to dissolve 4.30 ml. of stabilized 2,5-dimethoxytetrahydrofuran, 5.41 ml. of 18 Normal sulfuric acid and 0.5 gram of the sodium salt of para-toluene-sulfonic acid. This solution was stirred for 10 minutes at 90° F. whereby the DMTF became hydrolyzed to succinaldehyde. 153 grams of sodium sulfate and 2 grams of sodium bromide were then added and the composition was mixed for 20 minutes. There was then added 20 grams of sodium acetate and 27 ml. of formalin, the volume was then brought to one liter with water and the pH was adjusted to 4.8 at 80° F. The composition prepared was employed as a prehardener for photographic films containing gelatin-silver halide photographic emulsions thereon and was found to be an effective prehardener prior to the processing of the film in the developing baths. This prehardener composition had the unique property of hardening the gelatin emulsion at a low pH and was very effective within the pH range of 4-5.

*Example 2*

A solution was prepared in 600 ml. of water at 90° F. of 0.10 ml. of octyl alcohol, 4.30 ml. of stabilized 2,5-dimethoxytetrahydrofuran, and 5.41 ml. of 18 Normal sulfuric acid. This solution was mixed for ten minutes after which time 153 grams of sodium sulfate and 2.0 grams of sodium bromide were added. The solution was then stirred for 20 minutes, whereupon 20 grams of sodium acetate and 27 ml. of 37% formalin and sufficient water to make the final volume 1 liter were added. The pH was adjusted to 4.80. This solution exhibited a good prehardening effect and could usefully be employed without the build-up of polymeric dirt on the film or apparatus.

The stabilized compositions of my invention can be used in a number of photographic color processes, such as that described in Hanson and Vogt U.S. application Ser.

No. 209,263, filed July 11, 1962, now Patent No. 3,246,987. In using the prehardening compositions of my invention in such color processes, it is necessary only to treat the photographic material prior to color processing with an aqueous solution containing my stabilized tetrahydrofuran compound. The conventional photographic processing steps can then follow this initial prehardening treatment. One modification in the conventional color processing which can be employed is to elevate the temperature so that the speed of the processing is increased, as indicated above.

As illustrated above, the stabilized tetrahydrofuran compositions of my invention can be employed alone or together with other photographic processing compounds, including formaldehyde and the like. The compositions can also contain other compounds, such as alkali metal bromides, alkali metal sulfates, and supplemental stabilizing compounds, such as the alkali metal salts, e.g., sodium, potassium, etc., of aromatic sulfonic acids, such as benzenesulfonic, p-toluenesulfonic, salicylsulfonic, chlorobenzenesulfonic, etc., acids. The quantity of dialkoxytetrahydrofuran compounds used in the prehardening bath itself can vary, although I have found that about 0.5 to 50 grams per liter are sufficient. The stabilized tetrahydrofuran compounds of my invention can also be employed in conjunction with compounds having fog-inhibiting properties, such as those described in Graham U.S. application Ser. No. 351,218, filed Mar. 11, 1964. Typical antifoggant compounds described in the application, which are useful in my invention include N-methylbenzothiazolium-p-toluenesulfonate, as well as other water-soluble benzothiazolium salts, including those having other alkyl substituents on the nitrogen atom thereof (e.g., ethyl and the like). Also useful as antifoggants when used in conjunction with my tetrahydrofuran compounds are benzothiazolium salts containing two benzothiazole nuclei joined together through an alkylene radical attached through the nitrogen atoms thereof. Water-solubilizing acid anions comprise perchlorate, toluenesulfonate, etc. In general, the prehardening solutions containing both the

4  
tetrahydrofuran compounds of my invention and the benzothiazolium antifoggants can contain from about 1 to 200 mg. per liter of the benzothiazolium salt.

The invention has been described in detail with particular reference to preferred embodiments thereof, but it will be understood that variations and modifications can be effected within the spirit and scope of the invention as described hereinabove and as defined in the appended claims.

10 What I claim as my invention and desire secured by Letters Patent of the United States is:

15 1. A composition comprising a dialkoxytetrahydrofuran compound, formaldehyde, an alkali metal salt of an aromatic sulfonic acid and at least 0.025% by weight, based on the tetrahydrofuran compound, of a stabilizer selected from the class consisting of butylated hydroxy-

20 2. An aqueous photographic prehardener composition containing from 0.5 to 50 grams per liter of 2,5-dialkoxytetrahydrofuran, formaldehyde, and at least 0.01% by weight based on the said tetrahydrofuran compound of 2,6-di-tert.-butyl-p-cresol.

25 3. In a photographic prehardener composition containing from 0.5 to 50 grams per liter of 2,5-dialkoxytetrahydrofuran, and formaldehyde, the improvement comprising the use of 2,5-dialkoxytetrahydrofuran stabilized against the formation of peroxides with at least 0.01% by weight, based on the said tetrahydrofuran compound, of a stabilizer selected from the class consisting of butylated hydroxy-

30 hydroxyanisole and butylated hydroxytoluene.

#### References Cited

35 Lundberg, W. O.: Autoxidation and Antioxidants, New York, Interscience Publishers, 1962, vol. II, pages 498-503.

NORMAN G. TORCHIN, Primary Examiner.

C. E. DAVIS, Assistant Examiner.